

Oct. 19, 1937.

H. L. BROWNBACK

2,096,157

METHOD OF MAKING BEARINGS

Filed July 5, 1935



Inventor  
Henry L. Brownback

Attorney  
Alexander Dowell

## UNITED STATES PATENT OFFICE

2,096,157

## METHOD OF MAKING BEARINGS

Henry Lowe Brownback, Norristown, Pa.

Application July 5, 1935, Serial No. 30,000

4 Claims. (Cl. 22—204)

This invention relates primarily to bearings particularly for use in gasoline and other internal combustion engines, and the principal object thereof is to provide a novel bearing and method 5 of making same, the bearing consisting of lining steel or ferrous shells with bronze, copper, copper-lead mixtures, or brass, my novel method involving a step in which the molten copper of the bronze or brass (or a molten copper film alone) 10 is permitted to soak into the heated steel or ferrous shell for a sufficient length of time to permit penetration thereof an appreciable distance into the steel shell and to form on the shell a surface copper-iron alloy bonded with 15 the steel, to which alloy the bronze or brass which forms the material of the bearing lining will subsequently readily unite, thereby providing a novel bearing having a decidedly better bond between the shell and lining, the lining in fact having 20 penetrated and alloyed with the surface of the steel shell in much the same manner as carbon in case-hardening processes.

Another object of the invention is to provide a novel method of case-hardening the exterior 25 of the steel shell simultaneously with the depositing of the lining within the shell.

A still further object is to provide a bearing in which the lead constituent of the lining presents a spheroid structure rather than a crystal- 30 line structure in the finished lining, and can carry a much greater load.

In most cases the lining of steel shells with bronzes or brasses and particularly copper-lead mixtures high in lead has heretofore been accomplished by heating the steel shell in a non-oxidizing atmosphere to a temperature considerably higher than the melting point of the bronze, and by heating the bronze to a temperature higher than its normal melting point, and then 40 removing the shell from the furnace, adding a flux, and pouring the bronze in the shell. As soon as this is done the piece is cooled quickly or quenched to avoid precipitation of the lead. As the copper of the lining is in contact with the 45 steel for only a short time interval the penetration is very slight, and moreover the copper has a tendency to oxidize during pouring. The flux, if used in excess, also causes trouble.

Another process heretofore used consisted of 50 putting bronze in a shell which was sealed at both ends and which contained a volatile flux. The shell was then placed in a furnace and heated until the bronze became liquid, after which time it was placed in a machine and centrifuged into 55 contact with the walls of the shell. In this process the bronze likewise came into contact with the heated steel for only a short interval of time and at a temperature which is constantly lowering, often necessitating heating the shell and 60 bronze or copper hotter than the ideal tempera-

ture instead of having them in contact for a definite period of time at the ideal bonding temperature as the shell was necessarily quenched just as soon as the bronze was distributed as otherwise the lead would be also centrifuged into contact with the steel shell destroying the bond. This process was limited to the use of alloys fairly low in lead for the reason stated.

In my process the bronze or brass and the shell is preferably placed in a crucible of the type shown in my French Patent No. 747,334, sealed at both ends except for a small vent hole, and the shell or tube charged into a furnace. If the furnace has a non-oxidizing or reducing atmosphere it is not necessary to add a volatile de-oxidant in the crucible, shell, or other part to be coated, but if the furnace is of the ordinary combustion type a volatile chemical should be added to be volatilized by the furnace heat and displace the air in the crucible and thus provide a reduc- 20 ing atmosphere.

The crucible, containing the shell and lining material, is heated at a temperature of about 1975 to 2000° F. for a length of time sufficient to melt the bronze, brass, or other copper alloy or mixture, and the crucible then turned or rolled slowly for a sufficient period of time to bring the molten brass, bronze or copper mixture in contact with the walls of the heated steel shell for an appreciable period of time, varying ap- 30 proximately from 3 to 6 minutes, allowing the copper to soak into the steel, for an appreciable distance to form a surface copper-iron alloy forming a bonding medium, and a coating of copper adhering to the surface of the copper-iron alloy. 35 The copper is found to have penetrated into the steel in somewhat the same manner as carbon in case-hardening processes. Afterwards, the crucible is removed from the furnace and agitated thoroughly by shaking, rolling, or otherwise, to 40 mix the constituents of the brass, bronze, or lead copper mixture (which latter is a mechanical emulsion and not a true alloy) to break up finely and thoroughly mix the various constituents of the mixture. In the case of crucibles in which 45 the brass or bronze descends by gravity, the crucible subsequently is up-ended and plunged into water or other cooling medium so as to fix the brass or bronze and also to anneal the copper content; or in case the brass or bronze is to be 50 centrifuged in place, the crucible is put in a centrifuging machine, and as soon as the mixture is centrifuged, the crucible is quickly chilled to prevent the heavy portions of the mixture being displaced and to anneal the copper constituent. 55

The main feature of my process is the soaking of the copper into the steel for a definitely long period of time at an ideal temperature instead of the short periods employed in the other processes, for I have found that if the copper is not 60

in intimate contact at the necessary temperature for the necessary time period for forming this alloy the bonding is faulty, i. e., not deep enough.

I will explain the invention with reference to 5 the accompanying drawing which illustrates several practical embodiments thereof to enable others familiar with the art to adopt and use the same; and will summarize in the claims the essential features of the invention, and novel features 10 of construction for which protection is desired.

In said drawing:—

Fig. 1 is a vertical section through a crucible for coating a shell interiorly only.

15 Fig. 2 is a similar section showing the crucible up-ended as when being heated.

Fig. 3 is a vertical section through the crucible showing a steel shell therein for coating both interiorly and exteriorly.

20 In Fig. 1 the shell 1 is to be coated on its interior only, and the shell itself forms the outer casing of the crucible. In Fig. 1 the steel or other piece to be coated is designated by the reference character 4, and is in the form of a tubular shell 25 and may have annular recesses 1a at the ends of the bore therein to receive the lining material.

The actual process in the manufacture of the bearings can be divided into two general finishing classes, centrifugal and gravity. The general 30 principles underlying the bearing are the same in both cases, and the process of manufacture is as follows:

The steel shell 1 of the bearing is prepared and is carefully cleaned, preferably by pickling. After 35 this the lower end of the shell 1 is hermetically sealed by a plate 2. The shell is then passed through a copper sulphate bath and copper deposited either naturally or electrolytically on the shell. A central core 3 is placed in the shell 1 and is passed through an opening in the plate 2, the core being welded as at 3a or otherwise secured to the plate 2 to form a gas tight joint. Core 3 extends somewhat beyond the opposite end of the shell 1, and its extended end is closed by a 45 disk 4 when a tubular core is used which is welded as at 4a or otherwise secured to core 3, and this disk 4 is drilled with a very small escape hole 5 the use of which will be explained later. This core 3 is only used in the case of gravity cast 50 bearings, and in this case a container 6 which acts as a metal reservoir is hermetically secured to the shell at the end opposite the plate 2, and container 6 is closed at its outer end by a plate 7 welded or secured thereto so as to form a gas 55 tight joint, the plate 7 having an opening 1a therein provided with a removable cover. In place of the core 3 a solid graphite core might be used in which case a vent opening would be provided in the side of the reservoir 6.

60 At this point a volatile flux 8 such as salicylic acid is introduced into the shell through opening 1a in sufficient quantity to displace the air when the bearing is heated and maintain a non-oxidizing atmosphere in the bearing. The bearing metal 9 such as lead copper mixture or lead bronze 65 or other bronze or brass alloy is put into the reservoir 6 through the opening 1a and the cover hermetically sealed. All the above operations are performed while the shell and parts are cold.

70 The crucible thus formed is preferably up-ended so that the reservoir 6 is lowermost, as illustrated in Fig. 2, and is then charged into a furnace and heated up to a temperature of approximately 1975 to 2000° F. As the crucible begins 75 to heat and before any oxidation can take

place the flux material 8 put into the shell volatilizes and displaces the air which escapes through the small orifice 5 in the inner end of the core 3 and passes into the furnace. In case a furnace having a controlled atmosphere is used, the volatilizable flux 8 will not have to be put in the shell as the heat will cause the air to expand and the controlled atmosphere in the furnace will displace the air in the bearing.

After the crucible and the alloy metal 9 contained therein has reached the above desired temperature, part of the lead will flow from the lead bronze and will collect in the bottom of the reservoir 6 (Fig. 2); also the thin coating of copper which has been deposited as explained will form a 15 copper alloy with the steel or iron of the shell. The bearing is now brought into such a position, preferably by slow rolling, that the copper alloy of the bearing metal 9 comes in contact with the copper steel alloy formed on the surface of the 20 shell 1 and forms a further copper steel alloy which penetrates into the surface of the bearing.

This rolling process takes a certain length of time in practice from 3 to 6 minutes, in which time the necessary temperature must be maintained. The crucible is then removed from the furnace and violently agitated for approximately 25 20 seconds in order to thoroughly mix the molten lead and other metals with the molten copper of the bearing, and the crucible then plunged into a 30 cooling bath. This fixes or sets the lining, which in its molten state after having been agitated in the case of bearings containing a great deal of lead is found to be in fact a lead emulsion, and the lead in the resultant lining metal presents a 35 spheroid structure rather than a crystalline structure and hence can carry far greater loads than lead in a crystalline structure. By actual test my bearing has carried loads up to 4200 pounds as distinguished from 3000 pounds for bearings in 40 which the lead has a crystalline structure. Also microphotographs of my bearing disclose a more favorable steel copper alloy on the surface of the shell than is possible were the molten copper which is separated from copper lead alloy not 45 held at the constant necessary temperature in contact with the steel over the period of time above stated, that is, the period 3 to 6 minutes for soaking the separated copper into the iron or steel. This soaking step is impossible were a 50 steel shell simply heated to the required temperature and then molten copper lead or copper bronze alloy poured into the steel and the whole plunged into a cooling solution before the copper and lead have had time to separate.

Moreover in my process the shell may be coated as at 10 on its outer surface while cold with any known hardening compound, and charged into a furnace of the muffled type in which the flame does not contact directly with the steel. 60 In this case while the crucible is being raised to the desired temperature and while the copper is soaking into the steel from the inside, the hardening compound is soaking into the steel from outside, and when the bearing is plunged 65 into the cooling liquid to fix the copper lead or lead bronze emulsion on the inside the necessary chilling to harden the exterior of the shell simultaneously takes place giving a copper lead or bronze lead lining bearing, case-hardened on 70 its exterior.

The same process using a reservoir shown in Fig. 3 in which the reservoir 6x embraces the exterior as well as the interior of the shell 1, can be used to simultaneously coat the inside 75

and outside surfaces of the bearing, in case a copper lead or lead bronze surface is desired on both surfaces. In this case the sides of reservoir 6x are extended to meet the plate 2x which is 5 also extended beyond the side of shell 1. In this case the linings on the interior and exterior of the shell 1 will be of the same alloy. If different alloys are desired two separate reservoirs must be used, one similar to reservoir 6 of Fig. 1 10 and the other similar to reservoir 6x of Fig. 3, the latter reservoir embracing the former.

The same process omitting the core can be used to centrifuge the bronze into the steel shell, in which case the bearing in its molten state is 15 taken from the furnace and violently agitated as in the case of a gravity cast bearing so as to form the emulsion noted, and the crucible is put into a centrifugal machine and the copper lead or lead bronze alloy centrifuged into place, and 20 immediately cooled by a cooling spray. Hence I form a bearing surface of bronze or lead copper alloy firmly anchored to a ferrous or other backing or shell which alloy is not soldered but bonded to the shell by alloying a part of the copper 25 forming it directly to the shell.

It is to be understood that the invention is not limited to the constructions shown by way of example; and the process may be applied to objects of all forms, hollow or otherwise. Moreover, the 30 non-oxidizing medium or atmosphere may be produced by other means, for example by a vacuum, and my invention includes, as novel commercial products, any steel objects coated superficially, interiorly or exteriorly, with bronze or 35 brass by the use of my method.

I claim:—

1. The method of making lead copper alloy bearings or the like which consists in cleaning a ferrous shell; hermetically sealing one end thereof; treating the shell with copper sulphate; introducing lead copper alloy lining material into the shell; hermetically sealing a reservoir at the other end of the shell; providing a vent; heating the shell to a temperature which will cause the copper sulphate to form an initial copper-iron alloy 40 on the shell and melt the lining; up-ending the shell so that the reservoir is lowermost; collecting the molten lead constituent of the alloy in the bottom of the reservoir; tilting the shell 45 and rotating same slowly to cause the molten copper constituent to intimately contact with the copper-iron alloy on the shell for a sufficient length of time to penetrate the surface thereof and increase the copper-iron bond; violently agitating the shell to thoroughly emulsify the molten lead and copper constituents; up-ending the shell to bring the emulsified lining constituents 50 into lining position in the shell while the lead constituent is in spheroidal form; and quickly chilling the shell to set the lining.

2. The method of making lead copper alloy bearings or the like which consists in cleaning a ferrous shell; hermetically sealing one end thereof; treating the shell with copper sulphate; introducing a volatile flux into the shell which 55 will maintain a non-oxidizing atmosphere therein when heated; introducing lead copper alloy lining material into the shell; hermetically sealing a reservoir at the other end of the shell; providing a vent; heating the shell to a temperature which will volatilize the flux and will cause

the copper sulphate to form an initial copper-iron alloy on the shell and melt the lining; up-ending the shell so that the reservoir is lowermost; collecting the molten lead constituent of the alloy in the bottom of the reservoir; tilting the shell and rotating same slowly to cause the molten copper constituent to intimately contact with the copper-iron alloy on the shell for a sufficient length of time to penetrate the surface thereof and increase the copper-iron bond; violently agitating the shell to thoroughly emulsify the molten lead and copper constituents; up-ending the shell to bring the emulsified lining constituents into lining position in the shell while the lead constituent is in spheroidal form; and quickly chilling the shell to set the lining material.

3. The method of making lead copper alloy bearings or the like which consists in pickling a ferrous shell; hermetically sealing one end thereof; treating the shell with copper sulphate to deposit copper thereon; introducing lead copper alloy lining material into the shell; hermetically sealing a reservoir at the other end of the shell; providing a vent; heating the shell to a temperature of about 2000° F. to cause the copper sulphate to form an initial copper-iron alloy on the shell and melt the lining; up-ending the shell so that the reservoir is lowermost; collecting the molten lead constituent of the alloy in the bottom of the reservoir; tilting the shell and rotating same slowly to cause the molten copper constituent to intimately contact with the copper-iron alloy on the shell for a sufficient length of time to penetrate the surface thereof and increase the copper-iron bond; violently agitating the shell to thoroughly emulsify the molten lead and copper constituents; up-ending the shell to bring the emulsified lining material into lining position in the shell while the lead is in spheroidal form; and quickly chilling the shell to set the lining material.

4. The method of making lead copper alloy bearings or the like which consists in pickling a ferrous shell; hermetically sealing one end thereof; treating the shell with copper sulphate to deposit copper thereon; introducing a volatile flux into the shell which will maintain a non-oxidizing atmosphere therein when heated; introducing lead copper alloy lining material into the shell; hermetically sealing a reservoir at the other end of the shell; providing a vent; heating the shell to a temperature of about 2000° F. to volatilize the flux and to cause the copper sulphate to form an initial copper-iron alloy on the shell and melt the lining; up-ending the shell so that the reservoir is lowermost; collecting the molten lead constituent of the alloy in the bottom of the reservoir; tilting the shell and rotating same slowly to cause the molten copper constituent to intimately contact with the copper-iron alloy on the shell for a sufficient length of time to penetrate the surface thereof and increase the copper-iron bond; violently agitating the shell to thoroughly emulsify the molten lead and copper constituents; up-ending the shell to bring the emulsified lining material into lining position in the shell while the lead constituent is in spheroidal form; and quickly chilling the shell to set the lining material.

HENRY LOWE BROWNBACK.